# EUROPEAN PATENT SPECIFICATION

(11) **EP 0 752 619 B1**
(45) Date of publication and mention of the grant of the patent: **05.09.2001**
(21) Application number: 96420194.1
(22) Date of filing: 04.06.1996
(51) Int. Cl.: G03C 7/25

(54) **Improved dye imbibition printing blanks and matrix films**
Empfangs- und Matrizenfilms für Farbstoffimbibitionsverfahren
Films donneur et accepteur d'images colorées pour le procédé par imbibition de colorant

(30) Priority: 20.06.1995 US 367; 20.06.1995 US 355; 20.06.1995 US 356; 12.03.1996 US 614423; 12.03.1996 US 614413; 12.03.1996 US 614454
(43) Date of publication of application: 08.01.1997
(73) Proprietor: EASTMAN KODAK COMPANY, Rochester, New York 14650-2201 (US)
(72) Inventor: Bowman, Wayne Arthur, c/o Eastman Kodak Co., Rochester, New York 14650-2201 (US); Hagmaier, Charles Peter, c/o Eastman Kodak Co., Rochester, New York 14650-2201 (US); Manioci, Frank Dean, c/o Eastman Kodak Co., Rochester, New York 14650-2201 (US); Bogdanowicz, Mitchell Joseph, c/o Eastman Kodak Co, Rochester, New York 14650-2201 (US); Nelson, Roger Wayne, c/o Eastman Kodak Co, Rochester, New York 14650-2201 (US)
(74) Representative: Parent, Yves

(56) References cited:
- EP-A- 0 461 416
- US-A- 3 625 694
- US-A- 4 266 044
- US-A- 5 135 835

## Description

### Field of the Invention

This invention relates to a photographic imbibition dye transfer process and imbibition printing materials. It relates particularly to improved dye imbibition printing blanks with improved antistatic properties and reduced haze, and use of such materials in forming an imbibition print.

### Background of the Invention

The imbibition printing dye transfer process is well known. According to common procedures, a tanned colloid relief image is formed by imagewise exposure of a suitable light sensitive layer on a support, differentially hardening the colloid layer in accordance with the imagewise exposure, and removing the colloid from the support in inverse proportion to the amount of imagewise light exposure. The differential colloid hardening and removal is conventionally performed with a pyrogallol hardening developer as described, e.g., in U.S. Patent 2,837,430. For full color prints, three separate relief images corresponding to the blue, green, and red color records of the image being reproduced may be formed in separate blue, green, and red light sensitive matrix films by three separate exposures though a color negative film. The resultant colloid relief images are then dyed with yellow, magenta and cyan dyes, and the dye images transferred to an imbibition printing blank receiver film. In this manner imbibition printed colored dye images may be obtained which faithfully reproduce a colored subject. Imbibition printing blanks typically comprise a dye receiving layer on a support. Where the resulting image is intended to be viewed by light projection, such as in a motion picture film, a transparent film support is generally used.

The photographic industry has long recognized the need to provide photographic film and paper with antistatic protection to prevent the accumulation of static charges during manufacture and use. Such protection is advantageous in photographic elements as static charges can cause irregular fog patterns in photographic silver halide imaging emulsions. To prevent the problems arising from an accumulation of static charges, it is conventional practice to provide an antistatic layer (i.e., a conductive layer) in a photographic element.

A wide variety of antistatic layers are known for use in photographic elements. Such layers, however, have not previously been used with dye imbibibition printing blanks. As the visual dye image is transfered to an imbibition printing element blank rather than being formed directly in a silver halide emulsion imaging layer of the element, and as the back side of an imbibition printing element support bearing a dye receiving layer will be in contact with such dye receiving layer when the element is rolled up, such printing elements have different requirements as to antistatic protection needs. While image fog problems due to static charge buildup are generally not a problem with imbibition printing elements, such charges may attract dirt and dust to the printing element surface under high manufacturing and processing speeds which may result in the formation of "pinholes" in the processed imbibition printing blanks as well as a variety of handling and conveyance problems.

U.S. Patents 3,625,694; 3,958,995; and 3,898,088 disclose cationic (basic) mordants which may be used in dye imbibition printing blanks. Such mordants are suitable for use with anionic (acid) printing dyes. When using blanks containing a dye receiving layer comprising a cationic mordant and a hydrophilic colloid such as gelatin as a binder, there is a tendency for the blank to be brittle resulting in cracking and degradation of the transferred dye image.

The necessity for maintaining flexibility in film is obvious in view of the handling to which it is subjected in manufacturing and use. For example, films are flexed and bent during use in cameras, printers, projectors, and processing equipment. The brittleness of film is affected by both temperature and relative humidity, the latter being generally of greater practical importance. Below approximately 25 percent relative humidity, a significant change in film brittleness may occur with only a small change in relative humidity. The failures in film as a result of lack of flexibility may be of different types, depending upon the nature of the stress.

It has been suggested to include plasticizers in imbibition printing blanks and photographic elements to reduce brittleness. U.S. Patents 2,882,156 and 3,709,690 disclose blanks containing mordants and polymer latices as plasticizers. U.S. Patent 5,135,835 relates to heat developable photographic elements which contain a mordant, oil droplets and a polymer latex having a glass transition temperature (Tg) of 40°C or less for improving brittleness.

US 4 266 044 describes a receptor layer of a dye imbibition printing blank which may contain a cationic mordant, antistatic, softening orgents and polymer latices. Problems to be Solved

It would be desirable to improve the manufacturability of dye imbibition printing material and the image quality of imbibition prints.

Accordingly, it would be desireable to provide cationic mordanted imbibition printing element blanks with sufficient antistatic properties which enable high manufacturing and processing speeds without adversely affecting printed image qualities.

Additionally, often when polymer latices are added to a mordant layer containing a cationic mordant the layer becomes hazy due to incompatibility between the latex and the mordant. It would accordingly be further desirable to provide a polymeric plasticizer for use with cationic mordants which would not result in increased haze.

### Summary of the Invention

In one embodiment, this invention provides an improved dye imbibition printing blank comprising a support bearing on one side thereof a dye-receiving layer comprising a cationic mordant, and further comprising an antistatic layer substantially free of cationic polymers. In a preferred embodiment of the invention, the antistatic layer is provided on the opposite side of the support relative to the dye-receiving layer. Such antistatic layer provides improved antistatic properties which enable high manufacturing and processing speeds without adversely affecting printed image qualities.

In a preferred embodiment of the invention, printing blanks are provided wherein the dye-receiving layer comprises a cationic mordant, a hydrophilic colloid and a plasticizer polymer, wherein the plasticizer polymer is a latex polymer having a glass transition temperature below about 30°C comprising from about 2 to 20 wt% of units having a quaternary ammonium group. In a particularly preferred embodiment, the latex polymer comprises a vinyl co-polymer addition product of from about 50 to 98 weight percent of acrylic or methacrylic ester units, 0 to 48 weight percent of vinyl benzene units and 2 to 20 weight percent of the quaternary ammonium group containing unit. Use of such latex provides a dye imbibition printing blank substantially free of haze and brittleness.

### Brief Description of the Drawings

Figure 1 depicts the absorption spectrum of a preferred UV absorbing dye.

Figure 2 depicts the spectral characteristics of a HOYA U-340 filter.

Figure 3 is a graph depicting the Matrix Exposure Profile for matrix films having various UV dye optical densities.

Figure 4 depicts the sensitometric curves for matrix films having varying levels of UV absorber dye exposed to UV light resulting from Example 4.

Figure 5 is a graph depicting the Best Fit Contrasts of the curves of Figure 4 vs. UV dye concentration.

Figure 6 depicts the absorption spectra of the UV absorbing dyes used in Example 5.

Figure 7 depicts the sensitometric curves for the matrix films exposed to UV light resulting from Example 5.

### Detailed Description of the Invention

Dye imbibition printing blanks within the scope of one embodiment of this invention comprise a support bearing on one side thereof a dye receiving layer containing a cationic mordant, and further comprise an antistatic layer. In a preferred embodiment, in addition to the cationic mordant, the dye image receiving layer also comprises a hydrophilic colloid, and a plasticizer polymer.

Any antistatic conductive materials, excluding cationic polymers, such as those previously suggested for use with photographic elements may be used in the printing element antistatic layer in accordance with the invention. Such materials include, e.g., anionic polymers, electronic conducting non-ionic polymers, and electrically-conductive metal-containing particles such as metal halides or metal oxides in polymer binders. While antistatic compositions comprising a cationic polymer are also applicable for use with conventional photographic elements, such as the highly crosslinked vinylbenzyl quaternary ammonium polymer disclosed in U.S. Patent 4,070,189, such antistatic materials are excluded from the scope of the instant invention. Dyes intended for printing on the cationic mordant containing printing blanks of the invention are anionic and will transfer from the front dye-receiving side of the film to the antistat backing when such sides come into contact (such as in a rolled film) if the backing contains a catonic polymeric material such as quaternary ammonium polymer, resulting in dye stain. For the purposes of this invention, "substantially free of cationic polymers" is intended to apply to the absence of cationic polymers above trace or impurity levels.

Examples of suitable antistatic materials and layers include the following. U.S. Patent 3,033,679 discloses an antistatic layer comprised of an alkali metal salt of a copolymer of styrene and styrylundecanoic acid. Films having a metal halide, such a sodium chloride or potassium chloride, as the conducting material in a hardened polyvinyl alcohol binder are described in U.S. Patent 3,437,484. In U.S. Patent 3,525,621, the antistatic layer is comprised of colloidal silica and an organic antistatic agent such as an alkali metal salt of an alkylaryl polyether sulfonate, an alkali metal salt of an arylsulfonic acid, or an alkali metal salt of a polymeric carboxylic acid. An antistatic layer comprised of an anionic film forming polyelectrolyte, colloidal silica, and a polyalkylene oxide is disclosed in U.S. Patent 3,630,740 while U.S. Patent 3,681,070 describes a copolymer of styrene and styrene sulfonic acid as an antistatic agent. U.S. Patent 4,542,095 describes antistatic compositions comprising a binder, a nonionic surface-active polymer having polymerized alkylene oxide monomers, and an alkali metal salt. In U.S. Patent 4,916,011, an antistatic layer comprising a styrene sulfonate-maleic acid copolymer, a latex binder, and an alkyl-substituted trifunctional aziridine crosslinking agent are disclosed. Antistat layers comprising a polythiophene with conjugated polymer backbone in the presence of a polymeric polyanion compound are described in EP 554,588; EP 553,502; EP 564,911; DE 4,138,628.

Any of the wide diversity of electrically-conductive metal-containing particles proposed for use heretofore in imaging elements can be used in the electrically-conductive antistatic layer of this invention. Examples of useful electrically-conductive metal-containing particles include donor-doped metal oxides, metal oxides containing oxygen deficiencies, and conductive nitrates, carbides or borides. Specific examples of particularly useful particles include conductive TiO₂, SnO₂, Al₂O₃, ZrO₂, In₂O₃, ZnO, TiB₂, ZrB₂, NbB₃, CrB₂, MoB, Wb, LaB₆, ZrN, TiN, TiC, WC, HfN, and ZrC.

Metal oxides, and particularly vanadium pentoxide as described, for example, in Guestaux, U.S. Patent 4,203,769, are preferred for use in the dye imbibition printing elements of the invention. Antistatic layers containing vanadium pentoxide provide excellent protection against static and are highly advantageous in that they have excellent transparency and their performance is not significantly affected by changes in humidity. The use of metal oxide materials is further advantageous, as their antistatic properties allow the use of a protective overcoat layer such as a layer of cellulosic material to provide abrasion protection and/or enhance frictional characteristics while still providing acceptable antistatic performance.

Conductive fine particles of crystalline metal oxides dispersed with a polymeric binder have been used to prepare optically transparent, humidity insensitive, antistatic layers for various imaging applications. Many different metal oxides, such as AnO, TiO₂, ZrO₂, Al₂O₃, SiO₂, MgO, BaO, MoO₃, and V₂O₅, are disclosed as useful as antistatic agents in photographic elements or as conductive agents in electrostatographic elements in such patents as U.S. Patents 4,275,103; 4,394,441; 4,416,963; 4,418,141; 4,431,764; 4,495,276; 4,571,361; 4,999,276; and 5,122,445. Preferred metal oxides are antimony doped tin oxide, aluminum doped zinc oxide, and niobium doped titanium oxide, as these oxides have been found to provide acceptable performance characteristics in demanding environments.

Particular preferred metal oxides are antimony-doped tin oxide and vanadium pentoxide having good resistance to static discharge and no dye stain resulting from transfer of dye from front side to the back of the film. For high dye imbibition printing blank manufacturing and processing speeds (e.g., transport speeds above about 60 m/s), a surface resistivity of less than 10⁹ ohms per square is desired for the printing blanks to prevent static discharges during unwinding of the film and the buildup of static dirt during handling of the film.

Preferred binders which may be included in the antistatic layer of the printing blanks of the invention include vinylidene chloride-containing latexes and polyesterionomer dispersions, which can improve the integrety of the layer and the adhesion of the layer to the support. Polyesterionomer refers to polyesters that contain at least one ionic moiety. Such ionic moieties function to make the polymer water dispersable. These polymers are prepared by reacting one or more dicarboxylic acids or their functional equivalents such as anhydrides, diesters, or diacid halides with one or more diols in melt-phase polycondensation reactions well known in the art as shown in U.S. Patents 3,018,272, 3,929,489, 4,307,174 and 4,419,437. Examples of this class of polymers include, for example, Eastman AQ polyesterionomers manufactured by Eastman Chemical Company.

To provide protection of the antistatic layer, a protective overcoat may be applied thereon. The protective layer can chemically isolate the antistatic layer and also serve to provide scratch and abrasion resistance. The protective overcoat layers may be, e.g., cellulose esters, cellulose nitrate, polyesters, acrylic and methacrylic copolymers and homopolymers, polycarbonates, polyvinyl formal polymethyl methacrylate, polysilicic acid, polyvinyl alcohol, and polyurethanes. Such layers may be aqueous coated or organic solvent coated as appropriate.

The chemical resistance of the antistatic layer or an overcoat can be improved by incorporating a polymer cross-linking agent into the antistatic layer or those overcoats that have functionally crosslinkable groups. Cross-linking agents such as aziridines, carbodiimide, epoxys, and the like are suitable for this purpose.

A suitable lubricant may also be included in the antistatic layer or protective overcoat in order to provide desired friction performance to assure good transport characteristics during manufacturing and handling of the elements of the invention. Many lubricating agents can be used including higher alcohol esters of fatty acids, higher fatty acid calcium salts, metal stearates, silicone compounds, paraffins and the like. Aqueous dispersed lubricants are preferred as they may be directly incorporated into an aqueous antistatic or overcoat layer, thus avoiding the need for a separately applied lubricant layer. The aqueous dispersed lubricants of carnauba wax and stearates are preferred for their effectiveness in controlling friction at low lubricant levels and their excellent compatibility with aqueous overcoat polymer solutions.

Matting agents may also be included in the antistatic layer or overcoat thereon in order to improve transport properties of the elements of the invention on manufacturing, printing, processing, and projecting equipment. Such matting agents can also help prevent sticking between the front and back sides of the elements in a tightly wound roll. Matting agents may be silica, calcium carbonate, other mineral oxides, glass speres, ground polymers and high melting point waxes, and polymeric matte beads.

The antistatic layer may also contain a coating aid to improve coatability, including anionic or nonionic coating aids such as para-isononylphenoxyglycidol ethers, octylphenoxy polyethoxy ethanol, sodium salt of alkylaryl polyether sulfonate, and dioctyl esters of sodium sulfossuccinic acid, which coating aids are typically used at from 0.01 to 0.30 weight percent based on the total coating solution weight.

Cationic mordants for use in the dye receiving layer of the printing blanks in accordance with the invention are preferably quaternary ammonium and phosphonium mordants of the type described in U.S. Pats. 3,898,088 and 3,958,995. The cross-linked mordants of U.S. Pat. 3,958,995 are particularly preferred. Such mordants are generally of the formula: wherein A' represents units of an addition polymerizable monomer containing at least two ethylenically unsaturated groups; B' represents units of a copolymerizable α,β-ethylenically unsaturated monomer; Q is N or P; R', R", and R"' are independently carbocyclic or alkyl groups; M⁻ is an anion; a is from about 0.25 to 5 mole percent, preferably from about 1 to 10 mole percent; b is from about 0 to 90 mole percent, preferably from about 0 to 60 mole percent; and c is from about 10 to 99 mole percent, preferably from about 40 to 99 mole percent, for effective dye mordanting.

It is understood throughout this specification that any reference to a substituent by the identification of a group containing a substitutable hydrogen (e.g. alkyl, amine, aryl, alkoxy, heterocyclic, etc.), unless otherwise specifically stated, shall encompass not only the substituent's unsubstituted form, but also its form substituted with any other photographically useful substituents. Typical examples of photographic substituents include alkyl, aryl, anilino, carbonamido, sulfonamido, alkylthio, arylthio, alkenyl, cycloalkyl, and further to these exemplified are halogen, cycloalkenyl, alkinyl, heterocyclyl, sulfonyl, sulfinyl, phosphonyl, acyl, carbamoyl, sulfamoyl, cyano, alkoxy, aryloxy, heterocyclyloxy, siloxy, acyloxy, carbamoyloxy, amino, alkylamino, imido, ureido, sulfamoylamino, alkoxycarbonylamino, aryloxycarbonylamino, alkoxycarbonyl, aryloxycarbonyl, heterocyclylthio, spiro compound residues and bridged hydrocarbon compound residues. Usually the substituent will have less than 30 carbon atoms and typically less than 20 carbon atoms.

The hydrophilic colloid may be any of those generally employed in the photographic field, including, for example, gelatin, colloidal albumin, polysaccharides, cellulose derivatives, water-soluble polymer or copolymer including, but not limited to polyvinyl compounds, including polyvinyl alcohol and derivatives thereof, partially hydrolyzed poly(vinylacetate-co-vinylalcohol), hydroxyethyl cellulose, poly(acrylic acid), poly(l-vinylpyrrolidone), poly(sodium styrene sulfonate), poly(2-acrylamido-2-methane sulfonic acid), polyacrylamides. Copolymers of these polymers with hydrophobic monomers may also be used. Gelatin is a preferred hydrophilic colloid. This may be gelatin per se or a modified gelatin such as acetylated gelatin, phthalated gelatin, oxidized gelatin, etc. Gelatin may be base-processed, such as lime-processed gelatin, or may be acid-processed, such as acid processed ossein gelatin.

In a preferred embodiment of the invention, the dye-receiving layer of the printing blanks are hardened with a cross-linking agent. Various types of hardeners are useful in conjunction with elements of the invention. In particular, bis(vinylsulfonyl) methane, bis(vinylsulfonyl) methyl ether, l,2-bis(vinylsulfonyl-acetamido) ethane, 2,4-dichloro-6-hydroxy-s-triazine, triacryloyltriazine, and pyridinium, 1-(4-morpholinylcarbonyl)-4-(2-sulfoethyl)-, inner salt are particularly useful. Also useful are so-called fast acting hardeners as disclosed in U.S. Patents 4,418,142; 4,618,573; 4,673,632; 4,863,841; 4,877,724; 5,009,990; 5,236,822.

In a preferred embodiment, the dye receiving layer of the imbibition printing blanks of the invention include a plasticizer polymer latex. Such latex polymer are preferably water insoluble vinyl copolymers derived from any copolymerizable monomers, such as α,β-ethylenically unsaturated monomer (including two, three, or more repeating units) such as ethylene, propylene, 1-butene, isobutene, 2-methylpentene, 2-methylbutene, 1,1,4,4-tetramethylbutadiene, styrene, α-methylstyrene; monoethylenically unsaturated esters of aliphatic acids such as vinyl acetate, isopropenyl acetate, allyl acetate, etc.; esters of ethyleneically unsaturated mono- or dicarboxylic acids such as methyl methacrylate, ethyl acrylate, diethyl methylenemalonate, etc.; monoethylenically unsaturated compounds such as acrylonitrile, allyl cyanide, and dienes such as butadiene and isoprene. The particular monomer units and their proportions may be selected to achieve a desired glass transition temperature for the resulting polymer as is well known in the art.

For effective plasticizing, and as a distinguishing factor from cationic dye mordants, the plasticizer polymers of the invention have a glass transition temperature of about 30°C or lower, more preferably about 20°C or lower. The latex polymers comprise from about 2 tc 20 wt%, more preferably 2 to 10 wt%, of units having a quaternary ammonium group. Such units are preferably acrylic or methacrylic esters or amides to which the quaternary ammonium group is appended. A preferred class of ethylenically unsaturated monomers which may be used to form the remaining 80 to 98 wt% portion of the preferred vinyl polymers of this invention includes acrylic or methacrylic esters and vinyl benzenes.

In preferred embodiments of the invention, the units of the plasticizer latex polymer having a quaternary ammonium group are as defined in Formula I below, and in particularly preferred embodiments of the invention the plasticizer latex is of the Formula I. wherein A represents units derived from an acrylic or methacrylic ester monomer; B represents units derived from a vinyl benzene monomer; R₁ is H or methyl; L is -C(O)O-, -C(O)NH-, or an aromatic linking group such as phenyl; M is a C₁ to C₁₂ alkenyl linking group, which may be straight, branched, or cyclic; R₂, R₃, and R₄ are C₁ to C₆ alkyl groups; X⁻ is an anionic counterion such as CH₃SO₄⁻, Cl⁻, Br⁻, or I⁻; w is 50 to 98 weight percent; y is 0 to 48 weight percent; and z is 2 to 20 weight percent.

Representative plasticizer polymers in accordance with one embodiment of the invention include the following:
- PP-1: poly(ethylacrylate-co-styrene-co-2-(N,N,N-trimethylammonium) ethyl methacrylate methosulfate) 71/19/10 wt
- PP-2: poly(ethylacrylate-co-2-(N,N,N-trimethylammonium)ethyl methacrylate methosulfate) 90/10
- PP-3: poly(butyl acrylate-co-styrene-co-2-(N,N,N-trimethylammonium)ethyl methacrylate methosulfate) 71/19/10 wt
- PP-4: poly(methyl acrylate-co-2-(N,N,N-trimethylammonium)ethyl methacrylate methosulfate) 95/5 wt
- PP-5: poly(ethyl acrylate-co-styrene-co-2-(N,N,N-trimethylammonium)ethyl methacrylate methosulfate) 75/20/5 wt
- PP-6: poly(butyl acrylate-co-3-(N,N,N-trimethylammonium)propyl methacrylamide methosulfate) 90/10 wt
- PP-7: poly(butyl acrylate-co-4-vinyl-N-methylpyridinium methylsulfate) 90/10 wt
- PP-8: poly(butyl acrylate-co-p-N-(vinylbenzyl)-N,N,N-trimet:hylammonium chloride) 90/10 wt

The plasticizer polymers may be synthesized as set forth in the representative synthesis example described below or by using other well known vinyl polymer synthesis procedures.

The plasticizer polymer in accordance with the preferred embodiment of the invention must contain a quaternary ammonium group to give acceptable haze and coating solution stability. Plasticizer latices which contain anionic groups cannot be coated because the mordant layer coating composition coagulates upon the addition of latices containing an anionic group.

Matrix films for use with printing blanks in imbibition printing dye transfer processes typically comprise a support bearing a light sensitive layer containing a hydrophilic colloid (typically gelatin), visible light absorbing particles (typically carbon), a silver halide light sensitive emulsion, plus various photographic addenda to provide satisfactory stability, as well as coating aids necessary for suitable manufacture. Sensitizing dyes may be used in the matrix films to provide blue, green, and red light sensitivity for recording the blue, green, and red color record imagewise exposures. Separate matrix films designed to optimize sensitivity for particular color record exposures may be used, or alternatively identical pan-sensitive matrix films may be used for each of the blue, green and red exposures.

The imbibition printing blanks described above may contain further features and layers as are known in the art. Preferred supports for such blanks comprise transparent polymeric films, such as cellulose nitrate and cellulose esters (such as cellulose triacetate and diacetate), polycarbonate, and polyesters of dibasic aromatic carboxylic acids with divalent alcohols such as poly(ethylene terephthalate).

Photographic silver halide emulsion layers may also be included in the printing blanks of the invention. In a motion picture film blank, such a layer may be included between the support and the dye receiving layer as is known in the art in order to enable recording a sound track for the film in accordance with conventional motion picture sound track recording, exposing, and processing procedures. Alternatively, a sound track may be printed on the blank receiver as part of the imbibition printing process.

If desired, the printing blank of the invention can be used in conjunction with an applied magnetic layer, such as those described in Research Disclosure, November 1992, Item 34390 published by Kenneth Mason Publications, Ltd., Dudley House, 12 North Street, Emsworth, Hampshire P010 7DQ, ENGLAND.

### Plasticizer Polymer Synthesis Example

A latex copolymer having the composition 75 wt % ethylacrylate, 20 wt % styrene, and 5 wt % 2-(N,N,N-trimethylammonium) ethylmethacrylate methosulfate is prepared as follows: to a 500 ml addition flask was added 100 ml of distilled degased water, 1 ml of Igepal CO 730, 1 ml Ethoquad 0/12, 75 g of ethyl acrylate, 20 g of styrene, 6.3 g of 80 % aqueous solution of 2-(N,N,N-trimethylammonium)ethyl methacrylate, and 0.5 g of 2,2'-azobis(2-methylpropionamidine)dihydrochloride. The mixture was stirred under nitrogen. To a 1 L reaction flask was added 300 ml of degased distilled water, 1 ml of Igepal CO 730, 1 ml of Ethoquad 0/12 and 0.5 g of 2,2'-azobis(2-methylpropionamidine)dihydrochloride. The reaction flask was placed in an 80°C bath with stirring and the contents of the addition flask was added over a period of 30 minutes. The contents was stirred at 80°C under nitrogen for 3 hours. The condenser was then removed and the flask was heated to 90°C with a nitrogen purge for 1 hour to remove residual monomer. The flask was then cooled to give a translucent latex containing 24 % solids.

### Example 1

Coated dye imbibition printing blank supports were prepared as follows:

### Support 1

A 4.7 mil polyethylene terephthalate film support was coated on the backside with a layer containing a copolymer of styrene sulfonic acid sodium salt and 2-hydroxyethyl methacrylate 70/30 wt (182 mg/m²), a polymer latex of methyl acrylate, vinylidene chloride, and itaconic acid (15/83/02 wt%)(60 mg/m²) and Cymel 300 (melamine-formaldehyde resin crosslinking agent from American Cyanamide Co.)(18 mg/m²) and on the front side with a gel subbing layer containing poly(acrylonitrile-co-vinylidene chloride-co-acrylic acid) (14/80/6 wt%).

### Support 2

A 4.7 mil polyethylene terephthalate film support was coated on the backside with a layer containing Nalco 1115 (colloidal silica from Nalco Chemical)(404 mg/m²), a polymer latex of methylacrylate, vinylidene chloride, and itaconic acid 15/83/02 wt (135 mg/m²) and on the front side with a gel subbing layer.

### Support 3

A 4.7 mil polyethylene terephthalate film support was coated on the backside with a layer containing antimony-doped tin oxide (370 mg/m²) and Witcobond 232 (polyurethane from Witco Corp.) (125 mg/m²) and on the front side with a gel subbing layer.

### Support 4

A 4.7 mil polyethylene terephthalate film support was coated on the backside with a layer containing antimony-doped tin oxide (226 mg/m²) and a polymer latex of methyl acrylate, vinylidene chloride, and itaconic acid 15/83/02 wt (75 mg/m²) followed by a layer containing Witcobond 232 (899 mg/m²) and on the front side with a gel subbing layer.

### Support 5

A 4.7 mil polyethylene terephthalate film support was coated on the backside with a layer containing Witcobond 232 (899 mg/m²) and on the front side a gel subbing layer followed by a layer containing antimony-doped tin dioxide (296 mg/m²) and gelatin (52 mg/m²).

### Support 6

A 4.7 mil polyethylene terephthalate film support was coated on the backside with a layer containing Witcobond 232 and a polyaniline imine (1:1 ratio)(108 mg/m²) followed by a layer containing Elvacite 2041 (polymethylmethacrylate from DuPont) (1076 mg/m²) and on the front side a gel subbing layer.

### Support 7

A 4.7 mil polyethylene terephthalate film support was coated on the backside with a layer containing a polymer of N-vinylbenzyl-N,N,N-trimethylammonium chloride and ethyleneglycol dimethacrylate 93/7 wt (129 mg/m²) and a polymer of acrylonitrile, vinylidene chloride and N,N-dimethylaminoethyl methacrylate methosulfate 25.1/73.4/1.5 wt (194 mg/m²) and on the front side a gel subbing layer.

### Support 8

A 4.7 mil polyethylene terephthalate film support was coated on the backside with a layer containing a polymer of N-vinylbenzyl-N,N,N-trimethylammonium chloride and ethyleneglycol dimethacrylate 93/7 wt (129 mg/m²) and a polymer of acrylonitrile, vinylidene chloride and N,N-dimethylaminoethyl methacrylate methosulfate 25.1/73.4/1.5 wt (194 mg/m²) followed by a layer containing cellulose diacetate (2690 mg/m²). The front side was coated with a gel subbing layer.

### Support 9

A 4.7 mil polyethylene terephthalate film support was coated on the backside with a layer containing vanadium pentoxide (3.2 mg/m²) and Eastman AQ55D (polyesterionomer from Eastman Chemical Co.) (32 mg/m²). The front side of the support was coated with a gel subbing layer.

### Support 10

A 4.7 mil polyethylene terephthalate film support was coated on the backside with a layer containing vanadium pent:oxide (296 mg/m²) and Eastman AQ29D (polyesterionomer from Eastman Chemical Co.) (3.2 mg/m²) followed by a layer containing Witcobond 232 (899 mg/m²) and the front side was coated with a layer containing a gel sub well known in the art.

### Support 11

A 4.7 mil polyethylene terephthalate film support was coated on the backside with a layer containing Elvanol 71-30 (polyvinylalcohol from DuPont) (54 mg/m²), Volan (methacrylato chromic chloride from DuPont) (1.9 mg/m²) and potassium nitrate (5.4 mg/m²). The front side of the support was coated with a gel subbing layer.

### Support 12

A 5 mil polyethylene terephthalate film support was coated on the backside with a layer containing vanadium pentoxide (3.2 mg/m²) and a polymer latex of acrylonitrile, vinylidene chloride and acrylic acid 15/9/76 wt (2.4 mg/m²) followed by a layer containing Elvacite 2041 (1064 mg/m²). The front side of the support was coated with a gel subbing layer.

### Control Support

A 4.7 mil polyethylene terephthalate film support was coated on the backside with a layer containing Witcobond 232 (899 mg/m²) and on the front side with a gel subbing layer.

Dye imbibition printing blank Samples 1-12 and a Control Sample were made using corresponding Supports 1-12 and the Control Support as follows. Each support was coated on the front side with a layer containing silver bromoiodide emulsion (1940 mg/m² Ag), EDTA sodium salt (83.2 mg/m²), methylbensothiazolium chloride (10.1 mg/m²), gelatin (3500 mg/m²) and bisvinylsulfonylmethyl ether (75.6 mg/m²) followed by a layer containing polymer of copoly (N-vinylbenzyl-N,N,N-trimethylammonium chloride-co-ethyleneglycol dimethacrylate) 93/7 mole (861 mg/m²), Olin 10G surfactant (97.3 mg/m²), potassium nitrate (39.7 mg/m²), gelatin (2800 mg/m²), and a polymer methacrylate methosulfate 75/25/5 wt (280 mg/m²).

The surface electrical resistivity and the water electrode resistivity for certain of the above coatings were measured. The results are indicated in Table I below.

**Table I**

| Sample | Surface Electrical resistivity (ohm/square, 20% RH) | Water Electrode resistivity (ohm/square, 20% RH) |
|---|---|---|
| 1 | 2 X 10¹⁰ | |
| 2 | 6 X 10¹¹ | |
| 3 | 5 X 10⁸ | |
| 5 | | 1 X 10⁹ |
| 6 | | 1 X 10⁹ |
| 7 | 5 X 10⁹ | |
| 8 | | 4 X 10⁹ |
| 9 | 1 X 10⁹ | |
| 10 | | 1 X 10⁸ |
| 11 | >3 X 10¹⁴ | |
| 12 | | 1 X 10⁷ |
| Control | >3 X 10¹⁴ | 4 X 10¹¹ |

Desired resistivity values for surface electrical resistivity are less than about 10⁹ and for water electrode resistivity are less than about 10⁹, and especially less than about 10⁸ ohm/square. While all antistatic materials will improve resistivity levels to some extent, the metal oxide containing antistatic layers of Samples 3, 5, 9, 10, and 12 demonstrate especially preferable results. It is also noted the antistat in Sample 1 is not photographic development process surviving, and therefore not preferred.

An unwinding electrification test is used to determine if there is a "discharge" or "glow" in the unwinding nip of a roll of light sensitive film during production or handling. During this test a roll of film is unwound at a high speed. If there is a large separation charge, due to the fact that two dissimilar materials are being separated, the electric field in the unwind nip will be large. It can be large enough such that the air can no longer sustain the intense field and air breakdown will occur resulting in a static discharge. Such discharge can potentially be harmful to a light sensitive emulsion which may be used for recording a sound track in an imbibition printing blank. Table II shows the results of such an unwinding electrification test which was performed on Samples 7, 8, 11 and 12.

**Table II**

| Sample | Glow observed |
|---|---|
| 11 | yes |
| 7 | yes |
| 8 | yes |
| 12 | no |

Retransfer of dye from the printed front side of a dye imbibition print to the backside during storage in the roll can be a problem especially at high humidity and temperature. An antistatic backing layer can play an important part in this retransfer. To check for dye retransfer, the front sides of imbibition prints dyed with magenta dye M-1 were placed in contact with the backsides of each of Samples 1-12 and the Control Sample between two glass plates, and the assemblage was then placed in a chamber at 80 percent relative humidity and 38°C for four days. The backs of the undyed imbibition prints were then observed for the presence of transfered dye. The results are shown in Table III.

**Table III**

| Sample number | Dye present |
|---|---|
| 1 | no |
| 2 | no |
| 3 | no |
| 4 | no |
| 5 | no |
| 6 | no |
| 7 | yes |
| 8 | no |
| 9 | no |
| 10 | no |
| 11 | no |
| 12 | no |
| control | no |

Antistatic backings that contain a cationic polymeric material as in Sample 7 can result in dye retransfer as indicated above. Overcoating this antistat layer with a polymer as in Sample 8 may solve this retransfer problem, but poorer antistatic properties result.

In accordance with the most preferred embodiments of the invention, Samples 3, 5, 9, 10, and 12 meet the desired attributes of desired resistivity, no glow discharge and no dye retransfer. These examples all contain metal oxide antistats.

### Example 2

Dye imbibition printing blanks were prepared as follows:

| Component | Coverage |
|---|---|
| Top layer: | |
| Mordant: copoly(N-vinylbenzyl-N,N,N-trimethylammoniumchloride co-ethyleneglycol dimethacrylate) | 861 mg/m² |
| 93/7 mole ratio | |
| Olin 10G surfactant | 97.3 mg/m² |
| KNO₃ antistatic agent | 39.7 mg/m² |
| gelatin | 2799 mg/m² |
| plasticizer polymer PP-1 | 280 mg/m² |
| | |

| Bottom layer: | |
|---|---|
| EDTA sodium salt | 83.2 mg/m² |
| Methylbenzothiazolium chloride | 10.1 mg/m² |
| Gelatin | 3498 mg/m² |
| Bisvinysulfonylmethyl ether | 75.6 mg/m² |

### Support:

A 4.7 mil polyethylene terephthalate film support coated on the backside with a layer containing Elvanol 71-30 (polyvinylalcohol from DuPont) (54 mg/m²), Volan (methacrylato chromic chloride from DuPont) (1.9 mg/m²) and potassium nitrate (5.4 mg/m²).

Additional blanks were prepared substituting plasticizer polymers PP-2, PP-3 and PP-4 and comparative plasticizer polymers C-1, C-2 and C-3 for PP-1 at equal weights.
- C-1: poly(methyl acrylate)
- C-2: poly(ethyl acrvlate)
- C-3: poly(ethyl acrylate-co-styrene) 80/20 wt

The haze of each coating was measured after drying using a XL-211 Hazegard system manufactured by BYK-gardner which measures the transmitted light passed through a sample. The results are presented in Table IV below:

**Table IV**

| Plasticizer Polymer | %Haze |
|---|---|
| None | 1.5 |
| PP-1 | 1.4 |
| PP-2 | 1.4 |
| PP-3 | 1.4 |
| PP-4 | 1.2 |
| | |
| C-1 | 7.5 |
| C-2 | 2.9 |
| C-3 | 4.1 |

As demonstrated above, plasticizer polymers other than those in accordance with the preferred embodiments of the invention in the presence of the mordant in the coating composition can cause hazy coatings to occur upon drying. This difficulty is overcome by using the plasticizer latex of the preferred embodiments of the invention.

### Example 3

The effectiveness of plasticizer latex in accordance with the preferred embodiments of the invention at reducing brittleness was also demonstrated. A dye imbibition printing blank was made as described in Example 2, with PP-5 in place of PP-1 at the indicated coverages. The brittleness test performed provides for quantitatively measuring the brittleness of film by subjecting it to bending. By means of a wedge, the diameter of a film loop was constantly changed through gradually decreasing openings until a failure of the film resulted. The opening of the wedge at which the film failed is the measure of its brittleness. The film was conditioned at 15 percent relative humidity and 21°C before running the test. The smaller wedge opening before the onset of failure the more flexible the film.

**Table V**

| Example | Polymer level mg/m² | Brittleness (relative wedge opening at failure) |
|---|---|---|
| 2.1 (comparison) | 0 | 0.20 |
| 2.2 (invention) | 215 | 0.11 |
| 2.3 (invention) | 430 | 0.08 |

Table V shows the effectiveness of the plasticizer latex of the invention to give acceptable coatings with reduced brittleness.

## Claims

1. A dye imbibition printing blank comprising a support bearing on one side thereof a dye-receiving layer comprising a cationic mordant, wherein the printing blank further comprises an antistatic layer substantially free of cationic polymers.

2. A printing blank according to claim 1, wherein the antistatic layer is provided on the opposite side of the support relative to the dye-receiving layer.

3. A printing blank according to claim 1 or claim 2 wherein the antistatic layer comprises an anionic polymer, electronic conducting non-ionic polymer, metal halide or metal oxide.

4. A printing blank according to any one of claims 1-3 wherein the antistatic layer comprises a metal oxide and a polymer binder.

5. A printing blank according to claim 4, further comprising a protective polymeric overcoat layer on the antistatic layer.

6. A printing blank according to any one of claims 1-5, wherein the cationic mordant is a quaternary ammonium or phosphonium mordant.

7. A printing blank according to claim 6, wherein the cationic mordant is of the formula: wherein A' represents units of an addition polymerizable monomer containing at least two ethylenically unsaturated groups; B' represents units of a copolymerizable α,β-ethylenically unsaturated monomer; Q is N or P; R', P'', and R''' are independently carbocyclic or alkyl groups; M⁻ is an anion; a is from 0.25 to 10 mole percent; b is from 0 to 60 mole percent; and c is from 40 to 99 mole percent.

8. A printing blank according to any one of claims 1-7, wherein the dye receiving layer further comprises a hydrophillic colloid and a plasticizer polymer, wherein the plasticizer polymer is a latex polymer having a glass transition temperature below 30°C comprising from 2 to 20 weight percent of units having a quaternary ammonium group.

9. A printing blank according to claim 8, wherein the plasticizer polymer is a vinyl co-polymer and wherein the units having a quaternary ammonium group are acrylic or methacrylic esters or amides to which the quaternary ammonium group is appended.

10. A printing blank according to claim 9, wherein the plasticizer polymer is of the formula wherein A represents units derived from an acrylic or methacrylic ester monomer; B represents units derived from a vinyl benzene monomer; R₁ is H or methyl; L is -C(O)O-, -C(O)NH-, or an aromatic linking group; M is a C₁ to C₁₂ alkenyl linking group; R₂, R₃, and R₄ are C₁ to C₆ alkyl groups; X⁻ is an anionic counterion; w is 50 to 98 weight percent; y is 0 to 48 weight percent; and z is 2 to 20 weight percent.

11. A printing blank according to any one of claims 1-10, wherein the support is transparent.

12. A printing blank according to any one of claims 1-11, further comprising a silver halide emulsion layer for recording a sound track.

## Patentansprüche

1. Druckrohling für Farbstoffimbibitionsverfahren mit einem Träger, auf dessen einer Seite eine Farbstoffempfangsschicht angeordnet ist, die ein kationisches Beizmittel umfasst, wobei der Druckrohling eine Antistatikschicht umfasst, die im wesentlichen frei von kationischen Polymeren ist.

2. Druckrohling nach Anspruch 1, **dadurch gekennzeichnet**, dass die Antistatikschicht auf der gegenüberliegenden Seite des Trägers relativ zu der Farbstoffempfangsschicht angeordnet ist.

3. Druckrohling nach Anspruch 1 oder 2, **dadurch gekennzeichnet**, dass die Antistatikschicht ein anionisches Polymer, ein elektronisch leitendes, nicht ionisches Polymer, Metallhalogenid oder Metalloxid umfasst.

4. Druckrohling nach einem der Ansprüche 1 bis 3, **dadurch gekennzeichnet**, dass die Antistatikschicht ein Metalloxid und ein Polymerbindemittel umfasst.

5. Druckrohling nach Anspruch 4, **dadurch gekennzeichnet**, dass die Antistatikschicht des Druckrohlings mit einer schützenden Polymerschicht überzogen ist.

6. Druckrohling nach einem der Ansprüche 1 bis 5, **dadurch gekennzeichnet**, dass das kationische Beizmittel ein quaternäres Ammonium- oder Phosphoniumbeizmittel ist.

7. Druckrohling nach Anspruch 6, **dadurch gekennzeichnet**, dass dem kationischen Beizmittel folgende Formel zugrunde liegt: wobei A' die Einheiten eines additionspolymerisierbaren Monomers darstellt, das mindestens zwei ethylenungesättigte Gruppen umfasst; B' stellt die Einheiten eines copolymerisierbaren α-, β-ethylenungesättigten Monomers dar; Q ist N oder P; R', R" und R''' sind unabhängig carbozyklische oder Alkylgruppen; M⁻ ist ein Anion; a ist ein Wert zwischen 0,25 und 10 Molprozent; b ist ein Wert zwischen 0 und 60 Molprozent und c ist ein Wert zwischen 40 und 99 Molprozent.

8. Druckrohling nach einem der Ansprüche 1 bis 7, **dadurch gekennzeichnet**, dass die Farbstoffempfangsschicht ein hydrophiles Colloid und ein Weichmacherpolymer umfasst, dass das Weichmacherpolymer ein Latexpolymer mit einer Glasübergangstemperatur von unter 30°C ist und 2 bis 20 Gewichtsprozent von Einheiten umfasst, die eine quaternäre Ammoniumgruppe aufweisen.

9. Druckrohling nach Anspruch 8, **dadurch gekennzeichnet**, dass das Weichmacherpolymer ein Vinyl-Copolymer ist und dass die eine quaternäre Ammoniumgruppe umfassenden Einheiten Acryl- oder Methacrylester oder Amide sind, denen die quaternäre Ammoniumgruppe angehängt ist.

10. Druckrohling nach Anspruch 9, **dadurch gekennzeichnet**, dass dem Weichmacherpolymer folgende Formel zugrunde liegt: wobei A die von einem Acryl- oder Methacrylestermonomer abgeleiteten Einheiten darstellt, B stellt die von einem Vinylbenzolmonomer abgeleiteten Einheiten dar; R₁ ist H oder Methyl; L ist -C(0)0-, -C(0)NH- oder eine aromatische Verbindungsgruppe; M ist eine C₁ bis C₁₂ Alkenyl-Verbindungsgruppe; R₂, R₃ und R₄ sind C, bis C₆ Alkylgruppen; X⁻ ist ein anionisches Gegenion; w ist 50 bis 98 Gewichtsprozent; y ist 0 bis 48 Gewichtsprozent und z ist 2 bis 20 Gewichtsprozent.

11. Druckrohling nach einem der Ansprüche 1 bis 10, **dadurch gekennzeichnet**, dass der Träger transparent ist.

12. Druckrohling nach einem der Ansprüche 1 bis 11, **dadurch gekennzeichnet**, dass der Druckrohling zudem eine Silberhalogenidemulsionsschicht zur Aufnahme einer Tonspur umfasst.

## Revendications

1. Récepteur pour tirage par imprégnation de colorants comprenant un support dont l'une des faces est revêtue d'une couche réceptrice de colorant comprenant un mordant cationique, ce film récepteur comprenant aussi une couche antistatique quasiment exempte de polymères cationiques.

2. Récepteur pour tirage par imprégnation de colorants selon la revendication 1, dans lequel la couche antistatique est appliquée sur la face du support opposée à la couche réceptrice de colorant.

3. Récepteur pour tirage par imprégnation de colorants selon la revendication 1 ou la revendication 2, dans lequel la couche antistatique comprend un polymère anionique, un polymère non ionique ayant une conductivité électronique, un halogénure métallique ou un oxyde métallique.

4. Récepteur pour tirage par imprégnation de colorants selon l'une quelconque des revendications 1 à 3, dans lequel la couche antistatique comprend un oxyde métallique et un liant polymère.

5. Récepteur pour tirage par imprégnation de colorants selon la revendication 4, comprenant aussi une surcouche polymère de protection au-dessus de la couche antistatique.

6. Récepteur pour tirage par imprégnation de colorants selon l'une quelconque des revendications 1 à 5, dans lequel le mordant cationique est un mordant ammonium ou phosphonium quaternaire.

7. Récepteur pour tirage par imprégnation de colorants selon la revendication 6, dans lequel le mordant cationique répond à la formule : dans laquelle A' représente des motifs d'un monomère polymérisable par addition contenant au moins deux groupes ayant une insaturation de type éthylénique ; B' représente des motifs d'un monomère copolymérisable ayant une insaturation de type α,β-éthylénique ; Q représente N ou P ; R', R'' et R''' représentent séparément des groupes carbocycliques ou alkyle ; M⁻ est un anion ; a est compris entre 0,25 et 10 % en moles ; b est compris entre 0 et 60 % en moles ; et c est compris entre 40 et 99 % en moles.

8. Récepteur pour tirage par imprégnation de colorants selon l'une quelconque des revendications 1 à 7, dans lequel la couche réceptrice de colorant comprend aussi un colloïde hydrophile et un polymère plastifiant, dans lequel le polymère plastifiant est un latex de polymère ayant une température de transition vitreuse inférieure à 30 °C et comprenant 2 à 20 % en poids de motifs ayant un groupe ammonium quaternaire.

9. Récepteur pour tirage par imprégnation de colorants selon la revendication 8, dans lequel le polymère plastifiant est un copolymère de vinyle et dans lequel les motifs ayant un groupe ammonium quaternaire sont des esters ou amides acryliques ou méthacryliques auxquels le groupe ammonium quaternaire est rattaché.

10. Récepteur pour tirage par imprégnation de colorants selon la revendication 9, dans lequel le polymère plastifiant répond à la formule : dans laquelle A représente des motifs issus d'un monomère ester acrylique ou méthacrylique ; B représente des motifs issus d'un monomère vinylbenzène ; R₁ représente H ou un groupe méthyle ; L représente -C(O)O-, -C(O)NH-, ou un groupe de liaison aromatique ; M représente un groupe de liaison alcényle ayant 1 à 12 atomes de carbone ; R₂, R₃ et R₄ représentent des groupes alkyle ayant 1 à 6 atomes de carbone ; X⁻ est un ion complémentaire anionique ; w est compris entre 50 et 98 % en poids ; y est compris entre 0 et 48 % en poids ; et z est compris entre 2 et 20 % en poids.

11. Récepteur pour tirage par imprégnation de colorants selon l'une quelconque des revendications 1 à 10, dans lequel le support est transparent.

12. Récepteur pour tirage par imprégnation de colorants selon l'une quelconque des revendications 1 à 11, comprenant aussi une couche d'émulsion aux halogénures d'argent pour enregistrer une piste sonore.
